

July 23, 1963

D. A. YOUNG ET AL

3,098,473

CATHODIC PROTECTION OF INTERNAL COMBUSTION ENGINES

Filed Jan. 25, 1962



EFFECT OF CATHODIC PROTECTION OF ENGINE PARTS  
IN 16 HOUR ENGINE RUST TEST



FIGURE 2

DALE A. YOUNG INVENTORS  
GEORGE J. FARRIS

BY *David A. Roth*

PATENT ATTORNEY

1

3,098,473

CATHODIC PROTECTION OF INTERNAL  
COMBUSTION ENGINESDale A. Young, Roselle Park, N.J., and George J. Farris,  
Chicago, Ill., assignors to Esso Research and Engineering  
Company, a corporation of Delaware

Filed Jan. 25, 1962, Ser. No. 168,763

7 Claims. (Cl. 123—99)

This invention relates to a method and apparatus for inhibiting corrosion of internal combustion engines. In particular, the invention pertains to a sacrificial anode technique for protecting automotive engines against corrosion. Even more particularly, the invention pertains to the prevention of valve train assembly, e.g. hydraulic valve lifter rusting by the use of a sacrificial anode.

A full understanding of the invention may be had by referring to the following description and claims taken in conjunction with the accompanying drawing in which FIG. 1 shows a view of a rocker arm assembly with a zinc strip held in place with one of the hold-down bolts of said assembly, and FIG. 2 shows a graph of rust vs. humidity in an engine rust test.

For several years now hydraulic type valve lifters have been used in increasing members in automotive engines. Any rusting tendencies within the engine become significant since these tendencies affect the operation of the hydraulic valve lifters. Hydraulic valve lifters generally comprise a cylindrical body, within which is an axially slideable plunger. The most detrimental corrosion or rusting occurs at the parts of contact between the plunger and the interior of the lifter body. Corroded hydraulic valve lifters tend to stick and create noise as well as to promote the possibility of serious engine damage because of their improper operation.

In order to prevent this corrosion of hydraulic valve lifters, lubricating oil manufacturers have incorporated rust preventive chemicals in their oil formulations. However, the requirements of a modern, internal combustion engine also dictate that an effective motor oil formulation must also contain a detergent-inhibitor in order to suspend any sludge formed. Unfortunately, chemical rust inhibitors and detergent-inhibitors have been found to be somewhat antagonistic to each other. Thus, inclusion of a rust preventive compound and a detergent inhibitor compound detracts from the potential effectiveness of either one if used alone.

It has now been discovered and forms the substance of this invention, that the problem can be alleviated by the use of a sacrificial anode located properly within the engine. In the past, sacrificial anodes in the form of magnesium nickel alloy drain plugs were used, but with little success. The reason for this is believed to be that the sludge formed within the engine settles to the bottom of the crankcase thus forming a film on the surface of the drain plug. This film provided sufficient resistance to the galvanic circuit necessary in a sacrificial anode apparatus to effectively stifle galvanic action. Furthermore, it is believed that the drain plug is too far removed from the parts to be protected, i.e. the hydraulic valve lifters, to form a suitable galvanic couple with these parts.

The most informed current view of the major cause of corrosion within an internal combustion engine is that it is due to galvanic corrosion. By galvanic corrosion is meant the accelerated attack on metals which results from the flow of current between dissimilar metals in electrical contact in a liquid capable of conducting current. Conditions necessary for galvanic corrosion are that there be a combination of dissimilar metals having a potential difference when they are in a corrosive environment, an electrical connection between the dissimi-

2

lar metals so that electrons can flow from one metal to another and an ionized liquid capable of conducting current between the dissimilar metals. Since the waste exhaust products such as water and blowby gases which contaminate the lubricating system of an internal combustion engine are strongly ionic, it will be recognized that all the above-named conditions are present in an internal combustion engine. The term "dissimilar metals" is used in a very broad sense; thus, two types of steel might be dissimilar, i.e. a carbonized steel and a chromium steel, or cast iron or wrought iron can be sufficiently dissimilar to set up a galvanic couple. In a galvanic couple the flow of electrons is from the anode to the cathode. Thus, it is the anode part of the galvanic couple which tends to corrode. It is also known that the greater the surface area of the cathode relative to an anode, the more severe the corrosive effect on the anode.

Therefore, in order to protect the metal in a particular environment, it is known to provide an anodic material in that environment which is higher in a galvanic series than the material to be protected. In this case since steel or iron can be considered the material to be protected it should be the cathode and a sacrificial anode must be higher in the galvanic series. Suitable materials higher in the galvanic series than steel or iron include cadmium, zinc, magnesium, in that order. Although these are the preferred metals, it will be understood that other metals and metal alloys can be used as long as they are higher in the galvanic series than the metal to be protected in the specific environment under consideration. The metal to be protected then becomes a cathode and the metal higher in the galvanic series then becomes an anode and is commonly referred to as a sacrificial anode.

Another important factor in the use of a sacrificial anode is the location of such anode. Thus, preferably, the anode should be located as close as possible to the particular cathodic material it is desired to protect. For instance, when it is desired to protect against corrosion of hydraulic valve lifters, especially the tappet portion, the sacrificial anode should be located as close to such valve lifter as possible. The importance of location then is twofold, one aspect being to increase the effectiveness of the sacrificial anode and the other to eliminate the possibility of films, such as sludge, forming on the metal surfaces which could increase the resistance of the galvanic circuit to an extent sufficient to nullify the galvanic action. Since the hydraulic valve lifter assembly is located close to the top of an internal combustion engine both sludges and other film forming substances are constantly washed off the hydraulic valve lifter assembly surfaces. Also, since these substances are generally heavier with respect to the main body of oil they tend to find their way to the bottom of the automobile engine block.

In utilizing the sacrificial anode of this invention, two general techniques can be employed both of which are equally satisfactory. One of these is to attach a strip of the sacrificial anode metal to a convenient location near the hydraulic valve lifter assembly. In some instances this can present difficulties since the tolerances of valve lifter assemblies are quite close. A convenient place and one that was used in a specific embodiment of this invention is one of the holdown bolts for the rocker arm assembly. However, the sacrificial anode metal can be attached by any convenient technique such as a rivet, bolt, adhesive such as an epoxy resin and the like. The only critical limitation is that a complete metallic circuit for the electron flow must be maintained.

The other technique is to deposit a film of the sacrificial anode metal on, or near, the portion of the en-

gine that is most susceptible to corrosion and most in need of protection. Thus, various portions of the valve train assembly can be galvanized with a metal such as zinc, i.e. zinc plated push rods. Such galvanization or other deposition techniques such as vapor deposition will effectively avoid any problems caused by tolerance limitations in the design of the hydraulic valve train.

With reference to the drawing, rocker arm assembly 1 is shown rigidly attached to cylinder head 2 by means of holdown bolts 3 and 4. The upper portion of push rod 5 engages rocker arm 6 which is part of rocker arm assembly 1. Zinc strip 7 is rigidly attached to rocker arm assembly 1 by holdown bolt 3.

It will be understood that although particular mention has been made to the hydraulic valve lifters, it is possible to satisfactorily protect the entire valve train assembly. The valve train assembly includes the hydraulic valve lifter, push rod, rocker arm assembly, valve, valve spring and cam shaft.

The invention will be more fully understood by reference to the following example.

#### Example 1

In order to demonstrate the outstanding rust inhibition results obtained by using the sacrificial anode technique of the invention a series of tests was carried out in an ER4-99 rust test.

The ER4-99 rust test is designed to provide a method for rating automotive crankcase lubricants for their rust preventive qualities. This technique involves the continuous operation of a CLR engine at constant speed and load for 16 hours under conditions conducive to the formation of engine rust.

The test uses a single cylinder CLR Oil Test Engine equipped with standard carburetion, external water and oil cooling, and a screw mechanism to regulate blowby. The CLR engine is an abbreviation for the Cooperative Lubricant Research engine which is manufactured by the Laboratory Equipment Corp. (LABECO) of Indianapolis, Ind. The test procedure and conditions are fully described in a paper entitled, "Evaluation of Rusting Characteristics of Motor Oils" by D. A. Young and G. J. Farris presented at the 1961 SAE National Fuels and Lubricants Meeting at Houston, Texas on or about November 9, 1961.

In brief, each run lasts for a duration of 16 hours at any selected intake air humidity measured in terms of grains of moisture per pound of dry air. In this series of runs a commercial lubricating oil was used containing conventional detergent inhibitors, rust inhibitors, V. I. improvers and pour point depressants. In the engine which was unprotected by a sacrificial anode seven 16-hour runs were made. One run was made at an engine intake humidity of approximately 108 grains of moisture per pound of air. Two runs were made at an approximate humidity of about 111 grains of moisture per pound of air and four runs were made at a humidity of about 128 grains of moisture per pound of air.

A zinc strip approximately one inch wide by two and one-half inches long with a thickness of about 20 gauge was affixed to the rocker arm assembly of the CLR engine by means of a holdown bolt as illustrated in FIG. 1. Two 16-hr. runs were made in the engine protected with the zinc strip. One of such runs was made at a humidity of approximately 129 grains of moisture per pound of air and the other such run was made at a humidity of about 141 air grains of moisture per pound of dry air. For each run the push rods were polished

anew, new hydraulic valve lifters were installed, and fresh oil was used. The push rods and hydraulic valve lifters were rated for rust at the conclusion of each 16-hour run. The rating was made on the basis of the G.M. scale wherein 0 equals 100% heavy rust and 10 equals no rust at all. The results obtained are summarized in the FIG. 2 graph.

It can be seen from the graph that ordinarily as the amount of moisture increases the amount of rust within the engine also increases. For equivalent amounts of moisture in the engine intake, the series of runs where the engine was protected by the sacrificial anode, shows considerably less rust than comparable runs made with no anodic protection.

Although the invention has been described in its preferred form with a certain degree of particularity, it is understood that numerous changes in the details of operation and construction and the combination and arrangement of parts can be resorted to without departing from the spirit and scope of the invention as hereinafter claimed.

#### What is claimed is:

1. A method of protecting an oil-containing lubricating system of a metallic internal combustion engine against corrosion which comprises positioning a sacrificial anode within the oil of said lubricating system at a relatively sludge-free location sufficiently close to the metal part of said system desired to be protected to form a galvanic couple therewith, said sacrificial anode being composed of metal higher in the galvanic series than said metal part desired to be protected, and said relatively sludge-free location being chosen such that sludges normally formed within said lubricating system cannot deposit sufficiently on said sacrificial anode to prevent the flow of electrons and ions between said anode and said metal part desired to be protected.

2. A method according to claim 1, wherein said metal part desired to be protected is the hydraulic valve train assembly and wherein said sacrificial anode is located proximate to said hydraulic valve train assembly.

3. A method according to claim 1 wherein said protective metal is zinc.

4. A method according to claim 2 wherein said protective metal is zinc.

5. In combination with a metallic oil-containing lubricating system of an internal combustion engine, a cathodically protected hydraulic valve train assembly comprising a valve train assembly having a rocker arm assembly, and a sacrificial anode attached to said rocker arm assembly, said sacrificial anode being composed of metal higher in the galvanic series than any component metal in said hydraulic valve train assembly.

6. A method of reducing hydraulic valve lifter sticking in the lubricating system of a metallic internal combustion engine which comprises positioning a sacrificial anode composed of metal higher in the galvanic series than the metal of said hydraulic valve lifter proximate to said hydraulic valve lifter to thereby form a galvanic couple therewith and to reduce corrosion of the metallic parts of said valve lifter by cathodic protection.

7. A method according to claim 5, wherein said metal of said hydraulic valve lifter is iron.

#### References Cited in the file of this patent

#### UNITED STATES PATENTS

- |           |        |               |
|-----------|--------|---------------|
| 2,424,145 | Butler | July 15, 1947 |
| 2,425,424 | Jones  | Aug. 12, 1947 |
| 2,963,015 | Caris  | Dec. 6, 1960  |